

May 5, 1925.

1,536,399

L. KIRSCHBRAUN

## PROCESS OF MAKING FELTED, FIBROUS, WATERPROOF SHEETS

Filed July 18, 1918

3 Sheets-Sheet 1



Witness,  
S. G. Mann

May 5, 1925.

1,536,399

L. KIRSCHBRAUN

## PROCESS OF MAKING FELTED, FIBROUS, WATERPROOF SHEETS

Filed July 18, 1918

3 Sheets-Sheet 2



Witness,  
J. F. Mann,

Inventor,  
Lester Kirschbaum  
and L. Belknap.

May 5, 1925.

1,536,399

L. KIRSCHBRAUN

## PROCESS OF MAKING FELTED, FIBROUS, WATERPROOF SHEETS

Filed July 18, 1918

3 Sheets-Sheet 3



Witness,  
S. B. Mann

Inventor,  
Lester Kirschbaum  
Frank L. Belknap

~~AMM~~

Patented May 5, 1925.

1,536,399

# UNITED STATES PATENT OFFICE.

LESTER KIRSCHBRAUN, OF EVANSTON, ILLINOIS.

## PROCESS OF MAKING FELTED, FIBROUS, WATERPROOF SHEETS.

Application filed July 18, 1918. Serial No. 245,470.

To all whom it may concern:

Be it known that I, LESTER KIRSCHBRAUN, a citizen of the United States, residing in the city of Evanston, county of Cook, and State 5 of Illinois, have invented certain new and useful Improvements in Processes of Making Felted, Fibrous, Waterproof Sheets, of which the following is a specification.

This invention relates to improvements 10 in process of making waterproof felted fibrous sheets, and has among its salient objects to provide a process of making felted or sheeted waterproof product used as roofing or covering of various kinds and which 15 consists essentially of a mixture of fibre, a normally adhesive bituminous binder, and an emulsifying agent, formed into a tough, solid, dry body; to provide a process which obviates the necessity of using as a base, 20 prepared felt such as is used in the manufacture of asphalt shingles and similar elements; to provide a process of which the product may have a wide range as to its flexibility, rigidity, weight and toughness, 25 and in which product a substantial body portion thereof can be made from relatively cheap or waste material; to provide a process of the character referred to in which a substantial portion of the materials thereof 30 may be such waste products as sawdust, clay, and the like; to provide a process for forming a product of the character referred to in which the mixture may be fed in an aqueous vehicle or medium continuously to a 35 felting or sheet forming apparatus and there formed into a sheet, and pressed, coated, dried and cut into any desired shape or size, all as a continuous operation; and in general to provide certain other improvements in 40 processes of the character referred to.

In the drawings—

Figs. 1, 1<sup>A</sup> and 1<sup>B</sup> taken together indicate mere or less conventionally and diagrammatically, a paper making machine equipped 45 with instrumentalities for practicing the herein described process.

Referring to the drawings,—1 designates an emulsifier adapted to receive asphalt, or other bituminous binder, liquefied by heat, 50 an emulsifying agent such as clay, and water, and by proper agitation to emulsify the asphalt in the water. The emulsifier comprises a tank of any suitable construction, which is shown as provided with a rotating shaft 2, driven through gears 3 and 55 4 from any source of power. The shaft 2

carries a series of agitator arms 5 cooperating with stationary arms 6 secured to the side of the tank.

In preparing the emulsion, clay of a col- 60 liodal character is put in the emulsifier which has previously been charged with hot water, the proportions being such that a thick paste of doughy or viscous consistency is produced. Asphalt or other bituminous or 65 pitchy binder, while liquefied by heat, is then slowly stirred into the paste, and water is gradually added from time to time to maintain the viscous working consistency. 70 The added water is preferably warm or hot 75 so as to keep the mass substantially at the approximate melting point of the asphalt. The agitation of these several ingredients disperses the asphalt in a very fine state of division throughout the aqueous medium 80 containing the emulsifying agent. It is to be understood that emulsifying agents other than clay may be employed, provided an emulsion is produced, which is not of such sticky or adhesive character as to cause it 85 to adhere to the paper making instrumentalities.

This batch contained in the emulsifier can be delivered to a beater 7 through pipe 8 controlled by valve 9. The beater 7 is of 85 any construction adapted for converting fibrous stock fibre into pulp and is shown as provided with a suitable beating roll or rolls 10 and 11. The pulp which I use may be made from any suitable fibrous material 90 such as paper waste, tan bark, wood pulp, cotton waste, grassy fibres, and hemp. After the fibre is beaten to a pulp, the pulp is delivered by means of pipes 12 and 13 and 95 pump 14 to a stuff chest 15. This chest 15 is provided with a mechanical agitator 16 driven from any suitable source of power.

The emulsion instead of being delivered to the beater 7 may be delivered direct to the stuff chest through pipe 17 controlled by 100 valve 18. If the emulsion is delivered directly to the beater it is closely and thoroughly beaten into thorough admixture with the fibrous stock, and if it is delivered directly to the stock chest it is there mixed 105 with the stock in such a way as to thoroughly incorporate it with the latter. It will be desirable in many cases to add a filler to the mixture which may be of such relatively cheap materials as saw dust, ground cork or any suitable comminuted material. It 110 may be desirable to add more clay to the

stuff chest also. The mixture in the chest 15 is thinned to the desired consistency by adding as much water as desired through the pipe 19. The mixture should be sufficiently diluted with water to permit the stock to flow freely and the fibers to felt with each other, as is usual in the formation of a paper sheet. The various materials should be so mixed that the resulting stock shall be free of any tendency to be sticky or adhere to the machine. It may be here noted that when the emulsified composition is formed, the particles of the asphaltic or bituminous binder should be so thoroughly and finely dispersed through the aqueous paste that the particles of the binder be effectually separated from each other and surrounded by the clay and water. The operator may ascertain that the emulsification has been sufficient by manual manipulation. If properly emulsified it will have a smooth, soapy feeling and be free from any tendency to exhibit adhesiveness. By the use of the term "emulsion of an non-adhesive character" I refer to a composition having the characteristics hereinbefore referred to. The exact nature and character of emulsions is not entirely settled and various opinion have been expressed regarding the theory of emulsification. According to the present invention the asphalt, or analogous pitchy material, while in a melted fluid or semi-liquid condition, is dispersed in very fine particles throughout the aqueous vehicle so that the minute particles of asphalt are separated from each other and held out of contact with one another. As the expression has been used in the arts, the asphalt may be said to constitute the internal phase, and the water the external phase.

In any event, the composition, or dispersion, as I may term it, is non-adhesive and, for example, can be readily washed off the hands, or off machinery with water. However, when the water is evaporated or removed, the particles of asphalt again revert to their adhesive and sticky condition. While it is true that the asphalt may be solid or semi-solid at ordinary atmospheric temperatures, it is in a heated fluid or semi-liquid condition while being emulsified and resumes its normal solid or semi-solid consistency when the dispersion is cold, without apparently altering the dispersion of the asphalt particles so long as contained in the aqueous vehicle. It is to be noted that this dispersion is of such a character that when it is mixed with the fibrous stock and formed into a sheet, the asphalt undergoes no change in character or constitution through the use of chemicals or other re-agents.

After the bituminized stock is thoroughly mixed it is delivered to the sheet forming

mechanism through pipe 20 controlled by valve 21. The delivery end of the pipe 20 is provided with outlet 22 which is preferably the width of the sheet desired. The outlet 22 delivers the mixture to a flow box 23 from which it over-flows onto an endless travelling screen or fourdrinier wire 24, which is trained around rollers 25 and 26. Intermediate idler rollers may be provided as desired. The upper lap of the screen travels across table rollers 27. At either side the screen is provided with confining belts or deckles 28 as ordinarily. A dandy roll 29 may be yieldingly mounted as at 31, and below it is shown a supporting roll 30.

As shown in Fig. 1, the apparatus is broken away to reduce the size of the drawings, although the endless screen or wire is of sufficient length to allow the desired amounts of water to drain through the screen. To facilitate the removal of the water from the sheet, I have shown the usual suction boxes 32 and intermediate pressure rolls 33, an additional suction pipe 34 being provided to remove water if desired.

In forming, the sheet passes over the foraminated wire or screen on to a fabric felt 35, which is trained around a series of rolls 36 and driven from any suitable source of power. Presser rolls 37 may also be provided. The newly formed sheet *a* is threaded up over the felt 38 to press rolls 39 and thence up over guide rolls 40 and 41 to a series of drying rolls 42. The felt 38 serves to take up any surplus moisture and returns over rolls 43.

The felt 35 may be cleaned by means of rotating brushes 44 and suitable showers 45. The felt 38 can also be cleaned by brushes 46 and showers 47, and the screen by brushes 48 and showers 49. It will be understood however, that one of the important features of the present invention is that the mixture which is to be sheeted is of such character that it can be readily washed off of the various felts and will not stick thereto.

After the formed and dried sheet leaves the rolls 42 it passes through calendar rolls 50 to the coating mechanism 51, which is provided with delivery pipe 52 for the coating material such as ordinarily employed in the manufacture of prepared roofing, and presser rollers 53 which may be of any suitable construction. If granular faced roofing is being formed, the coated sheet can be fed beneath hopper 54 containing suitable granular material so as to cover the face of the roofing. The sheet then coated and covered with granular material is passed between presser rolls 55 and thence over cooling rolls 56 to slitting knives 57 carried by roll 58. The sheet which is now severed longitudinally may be cut transversely to form shingles or shingle strips by passing

through transverse knives 59 carried by rollers 60. It is to be understood of course that these knives and rolls are so geared as to operate synchronously. The shingles or shingle strips are then carried away by travelling conveyor belt 61.

The apparatus here shown is adapted for making shingles or shingle strips of prepared roofing such as asphalt shingles and 10 the like, but it is to be understood that the sheet after having been formed may be treated in any desired manner, such for example, as having a design printed thereon, etc., for use as flooring.

15 It may be desirable in certain instances to put a granular facing over the sheet and dispense with the coating. This may be done by impressing granular material on the sheet through the hopper 61' while the 20 sheet is still in sufficiently plastic condition to permit the granular or powdered material to become partially embedded in and adhere to the sheet. In other cases it may be desirable to give a color or luster to the roofing 25 and this can be accomplished by covering the granular facing of the roofing after it is applied with a film of silicate of soda and a pigment or dye, the pigment or dye giving the desired color.

30 In order to more readily practice the invention the following proportions of ingredients have been found satisfactory in the manufacture of fully saturated roofing felt. To 33 parts dry weight of fibrous stock is 35 added an emulsion composed of 55 parts by weight of asphalt emulsified with 12 parts by weight of colloidal clay contained in an aqueous vehicle. It will be understood that these proportions will vary depending upon 40 the nature of the stock and the degree of saturation with asphalt desired in the finished sheet. Of course, during the sheet-forming operation the particles of binder will be distributed among and deposited on 45 the fibres in the sheet during the felting of the same.

By the term "bituminous" applied to the binder I mean to include those natural and 50 artificial asphalts or other residual products of petroleum, coal tar pitch, or other pitches and analogous fusible pitchy or resinous substances, which are normally adhesive or of such an adhesive character that they will not normally in an aqueous medium pass 55 over a paper forming machine without sticking thereto unless they are converted to a non-adhesive state.

I claim as my invention:

1. The process of making a felted water 60 resistant sheet consisting in so treating a normally adhesive bituminous water proof binding medium as to render it non-adhesive, mixing it with a fibrous pulp in an aqueous vehicle, passing the mixture over 65 a paper forming machine and felting the

fibres, and drying the sheet to cause the binding medium to resume its adhesive condition.

2. The process of forming a water resistant 70 felted sheet, consisting in treating a normally adhesive bituminous binder to form a non-adhesive dispersion, comprising the binding material suspended in finely divided particles in water containing an emulsifying agent, then mixing the dispersion with fibre held in an aqueous vehicle, then felting the stock so formed on a paper forming machine and removing the water to restore the binder to its adhesive condition. 80

3. The process of forming a water resistant 85 felt which consists of liquifying a bituminous binder with heat, forming an aqueous paste of water and colloidal clay, then mixing the liquified binder with said paste to produce a non-adhesive dispersion in which the binder is in a state of fine dispersion, mixing said dispersion with fibrous material in an aqueous vehicle, then felting the stock so formed on a paper forming machine, and finally removing the water to restore the binder to its adhesive condition. 90

4. The process of forming a water resistant 95 felted sheet consisting in liquifying a bituminous binder by heat, liquifying colloidal clay with water to form a paste, mixing said binder and said paste to produce a non-adhesive emulsion or dispersion in which the binder is finely dispersed, mixing such dispersion with fibrous material contained in an aqueous vehicle in sufficient proportion 100 finally to produce a water resistant sheet, then felting the stock so formed on a paper forming machine, and finally drying said sheet. 105

5. The process of making a felted water 110 resistant sheet consisting in so treating a normally adhesive water proof binding medium to form an emulsion containing the binder, an emulsifying agent and water so as to render the binder non-adhesive, mixing it with a fibrous pulp in an aqueous vehicle and in sufficient proportion finally to produce a substantial saturation of the sheet therewith, passing the mixture over a paper forming machine and felting the fibres, and drying the sheet to cause the binding medium to resume its adhesive condition. 115

6. The process of forming a water resistant 120 felted sheet, consisting in mixing a water proof adhesive bituminous binder, an emulsifying agent and water to produce a non-adhesive composition, mixing fibrous material in an aqueous vehicle with such proportion of said composition finally to produce a substantial saturation of said sheet with said binder, then felting the stock so formed on a paper forming machine, and finally removing the water to restore the 125 binder to its adhesive condition. 130

7. The process of forming a water resistant felted sheet on a paper forming machine, consisting in mixing a water proof adhesive bituminous binder with colloidal clay to 5 form an emulsified composition in which the binder is held in finely divided particles out of contact with one another, then mixing this composition with fibrous material in an aqueous vehicle, then felting the 10 stock so formed on a paper forming machine and removing the water to permit the binder to reassume its adhesive state and unite with the fibres.
8. The process of forming a water resistant 15 felted sheet, consisting in treating an adhesive bituminous binder to form a non-adhesive dispersion comprising the binder suspended in finely divided particles in emulsified form, mixing said dispersion with 20 a sufficient quantity of fibre, to permit of felting, held in an aqueous vehicle, then felting the stock so formed on a paper forming machine and removing the water for restoring the binder to its adhesive condition.
9. The process of forming a water resistant 25 felted sheet, consisting of so treating a bituminous binder with water and an agent as to form a non-adhesive composition in which the binder will be held in finely dispersed particles out of contact with one another, mixing this composition with a fibrous 30 stock in an aqueous vehicle, feeding said mixture to a paper, or web forming mechanism and forming a felted sheet while the 35 binder is still in a non-adhesive condition and removing the water and causing the binder to reassume its adhesive state and unite with the fibres.
10. The process of forming a water 40 resistant felted sheet, consisting in making a non-adhesive emulsified dispersion from an adhesive water proof bituminous binder, an emulsifying agent and water, thoroughly incorporating this dispersion with a fibrous 45 pulp, flowing the stock so formed while the dispersion is still in a non-adhesive condition over mechanism for felting the fibres, and then removing the water from and drying the sheet so formed whereby said binder 50 will reassume its adhesive condition and unite with the fibres.
11. A process of forming a water resistant 55 felted sheet on a paper forming machine, consisting in mixing a normally adhesive bituminous binder with an emulsifying agent to form an emulsified composition in which the binder is held in finely divided particles out of contact with one another, then mixing this composition with fibrous 60 stock, then felting the stock so formed on suitable felting machinery, removing the water, the proportion of binder being in excess of 10% by weight of the finished product.
12. A process of making a felted water re- 65 sistant sheet, consisting in so treating a normally adhesive bituminous binder as to render it non-adhesive, mixing the same with a fibrous pulp in an aqueous vehicle, passing the mixture thus produced over a paper forming machine so as to cause the fibers to interlock and interlace, and merely by the removal of water and the application of heat causing the bitumen to become adhesive and unite with the fibres. 70
13. A process of making a felted water resistant sheet, consisting in so treating a normally adhesive bituminous binder as to render it non-adhesive by causing the particles to be held apart from each other by the action of a suitable material, mixing such bitumen while non-adhesive with fibrous pulp in an aqueous vehicle, passing such mixture over a paper forming machine so as to cause the fibres to interlock and interlace, and merely by removing the water and application of heat to cause the binder to take an adhesive form and unite with the fibres. 75
14. A process of making a felted water resistant sheet, consisting in so treating a waterproof bituminous binder as to render it non-adhesive, mixing the same with fibrous pulp in an aqueous vehicle, holding the particles of the binder apart in an aqueous vehicle by the action of a third substance, passing the mixture over a paper forming machine so as to cause the fibres to interlock and interlace and then removing the water. 80
15. The herein described process, which comprises mixing in water paper-making stock and an emulsion containing waterproofing material and clay, and forming on a paper-making machine a sheet from said mixture. 85
16. The herein described process, which comprises mixing in water paper-making stock and an emulsion containing bituminous waterproofing material and clay, and forming on a paper-making machine a sheet from said mixture. 90
17. The herein described process, which comprises mixing in water paper-making stock and an emulsion containing asphalt and clay, and forming on a paper-making machine a sheet from said mixture. 95
18. The herein described process comprising mixing in water, paper-making stock and an emulsion containing waterproof material at least semi-solid at normal atmospheric temperatures and clay, and in forming on a paper-making machine a sheet from said mixture. 100
19. The herein described process, which consists in producing an emulsion by heating a normally adhesive waterproof binder solid at atmospheric temperatures to liquify the same, in emulsifying said liquified binder with an emulsifying agent 105
- 125
- 130

and water, so that the binder constitutes the internal phase of the emulsion, in mixing said emulsion with paper-making stock, in forming on a paper-making machine a sheet from said mixture, and in causing the binder to resume its normally adhesive condition in said sheet.

20. The herein described process, which comprises mixing in water, paper-making stock and a non-adhesive emulsion containing waterproofing material emulsified with clay, and forming on a paper-making machine a sheet from said mixture.

21. The herein described process, which

comprises mixing in water, paper-making stock and a non-adhesive emulsion containing bituminous waterproofing material emulsified with clay, and forming on a paper-making machine a sheet from said mixture.

22. The herein described process, which comprises mixing in water, paper-making stock and a non-adhesive emulsion containing asphalt and clay, and forming on a paper-making machine a sheet from said mixture.

LESTER KIRSCHBRAUN.